

J. A. W. PINE & W. B. RUGGLES.  
ART OF TREATING ASPHALT.  
APPLICATION FILED NOV. 6, 1909.

1,057,667.

Patented Apr. 1, 1913.



WITNESSES

John B. Ruggles  
Emmett J. Peck

INVENTORS

J. A. W. Pine  
W. B. Ruggles  
BY  
Drell, Warfield & Drell  
ATTORNEYS

# UNITED STATES PATENT OFFICE.

JAMES A. W. PINE AND WILLIAM B. RUGGLES, OF NEW YORK, N. Y.

## ART OF TREATING ASPHALT.

1,057,667.

Specification of Letters Patent.

Patented Apr. 1, 1913.

Application filed November 6, 1909. Serial No. 526,869.

*To all whom it may concern:*

Be it known that we, JAMES A. W. PINE and WILLIAM B. RUGGLES, citizens of the United States, residing at New York city, in the county of New York and State of New York, have invented certain new and useful Improvements in the Art of Treating Asphalt, of which the following is a full, clear, and exact description, such as will enable others skilled in the art to which it appertains to make and use the same.

This invention relates to the art of treating asphalt and, more specifically to the art of preparing asphalt paving material from crude Trinidad asphalt.

One of the objects thereof is the practical and economical handling of crude Trinidad asphalt or an asphalt of that character and general composition.

Another object thereof is to provide an asphalt paving material prepared in a simple and inexpensive manner.

Other objects will be in part obvious and in part pointed out hereinafter.

The invention accordingly consists of the several steps and the relation and order of each of the same with respect to one or more of the others thereof, as will be set forth in the following description, and the scope of the application of which will be indicated in the appended claims.

The drawing graphically illustrates the several steps of the art, the dotted lines indicating that certain of said steps may be entirely omitted, or occur in altered relation to the other steps thereof.

In order to render certain features of this invention more readily and fully understood, it may be here noted that natural asphalt of the class known as Trinidad asphalt is a natural deposit of approximately the following composition: water (probably sea-water), 27-30%; bitumen, 37%; mineral matter (clay and fine sand), 33-38%. There is also present an appreciable quantity of various soluble salts. It has been found desirable in practice to reduce the high percentage of water to a minimum, as the retention thereof adds greatly to the expense of shipment of the asphalt from the place of deposit to the point at which it is desired to make use of the same. It has further been found that the presence of soluble salts has a deteriorating effect upon asphalt pavements, being, in fact supposed to be the

cause of the so-called rotting of pavement having that material as a cementing agent. If it be attempted to dispel the said water from the crude asphalt by the application of heat it will be found a very tedious and costly operation and, moreover, as relatively high temperatures will be found necessary, because of the natural non-conductivity of the asphalt, there will result a tendency to scorch or burn the asphalt itself and thereby impair many of the valuable qualities thereof.

By this invention sufficiently thorough drying is attained, soluble salts, if desired, may be washed out and a paving material of superior quality is produced; moreover these beneficial results are reached in a simple, practical, and economical manner.

The various steps employed in following out the art of the present invention will now be described.

First the crude asphalt is ground, pulverized or otherwise comminuted to any desired degree of fineness by the aid of any suitable means, after which it is agitated in water to separate therefrom, if desired, soluble salts inherent in its composition. It is to be understood that the washing may be accomplished without agitation, and, if found desirable, by the use of solvents other than water. The washed or unwashed asphalt is then dried either by evaporation in the atmosphere or by exposure to heat in any drier suitable for that purpose. Preferably a mechanical drier is employed because of its applicability to this kind of heating. It has been found that when the pulverized asphalt is dried by artificial heating a degree of temperature is liable to be reached at which there is a tendency for the granular particles to become sticky, adhere and run together. This is found to occur at and above 150° F., which temperature may not be sufficiently high to efficiently and expeditiously dispel the moisture. The addition of a small percentage of a refractory powdered substance, as marl, to the granular asphalt, either precedent to or simultaneously with its introduction into the drier serves to effectively preclude the adhesion of the particles thereof and to render possible the raising of the temperature to or slightly above the boiling point of water, whereupon a large percentage of the moisture is quickly and cheaply evaporated.

The introduction of powdered marl or other similar substance is otherwise advantageous, in that it prevents the particles of the asphalt from sticking together in transit, under varying conditions of temperature, when the said material is shipped in bulk or packed in bags. As a next step in carrying out the said art of preparing paving material, suitable sand is heated, as in rotary drums, to a temperature varying from about 350° to 10 500° F., and this hot sand together with a percentage of stone dust or other fine mineral matter is dumped into a mechanical mixing machine into which is introduced, 15 in proper proportion, cold, comminuted, (washed if desired) dried Trinidad asphalt. In practice about 15% of this asphalt is mixed with 85%, more or less, of the sand or mineral matter, which has been heated 20 to a temperature of from 350° to 500° F. Thereupon there ensues a thorough and uniform mixing of the two granular substances and at the same time the heat imparted to the cold asphalt by the much larger quantity 25 of hot sand will very quickly drive off whatever moisture there may be still remaining in the asphalt. Fluxing material, usually petroleum residuum of from 14° to 22° Baumé gage, in either hot or cold condition, is added before, simultaneously with, or immediately after the cold granular asphalt is introduced into the mixer containing the hot sand and after a few minutes 30 mixing in the machine a very uniform and superior asphalt paving material is obtained. The heat of the entire mass can be 35 readily maintained at or above 325° F., at which temperature the material is in suitable condition for hauling to and laying on the street.

It will be understood that by the addition of a suitable solvent to comminuted (washed if desired), dried Trinidad asphalt an asphaltic cement is obtained which may be 40 used for paving and other purposes without the necessity of heating either the asphalt tended to be mixed and this is accomplished in a very simple and inexpensive manner, in a very simple and inexpensive manner, 45 without resorting to the use of extensive and costly plants such as are necessitated by the methods now generally employed in the refining and utilization of Trinidad asphalt. In this connection, it will be noted, 50 that heretofore Trinidad asphalt has been used in a hot fluid condition, with the addition thereto of various mineral substances, to form a bituminous concrete. The present invention comprehends the preparation 55 of a dry granular or powdery bituminous cement which may be readily shipped in bags or in bulk. This cement may be heated, or treated with a solvent in order to bring out its cementitious qualities and it 60 is then only necessary to mix in proper

quantities with suitable mineral matter to obtain an inexpensive and durable bituminous concrete. It will therefore be seen that the present invention is well adapted to attain the advantages hereinbefore set forth, in a simple, efficient, and inexpensive manner. 70

It is to be understood that by the term Trinidad asphalt, is meant, in the present specification and claims, not only that composition of bitumen and mineral matter which is at the present time principally obtained from the so-called "pitch lake" in the island of Trinidad, British West Indies, but also any bituminous substance having approximately like composition and characteristics. It is to be noted that the expressions "cold" and "at ordinary temperatures" occurring in the claims are employed to denote the fact that the dry granular asphalt is mixed at its existing temperature, without preheating, with the preheated mineral matter and fluxing agent. 80

As the above art could be carried out by means of various kinds of apparatus and could be varied without departing from the scope of this invention, and as many features of the above art are of independent value, it is intended that all matter contained in the above description shall be interpreted as illustrative and not in a limiting sense. It is also to be understood that the language used in the following claims is intended to cover all of the generic and specific features of the invention herein described and all statements of the scope of the invention, which, as a matter of language, might be said to fall therebetween. 95

Having described our invention, what we claim as new and desire to secure by Letters Patent is:

1. The improvement in the art of preparing paving material which comprises comminuting crude Trinidad asphalt, agitating in water to remove soluble salts, and then subjecting same to a drying process embodying an application of heat at a sufficiently low temperature to maintain the asphalt in a granular condition. 110

2. The improvement in the art of preparing paving material which comprises comminuting crude Trinidad asphalt, adding thereto an agent adapted, under ordinary conditions of handling at temperatures below a certain predetermined temperature, to prevent adhesion of the particles thereof and then subjecting the mixture to a drying process embodying an application of heat at a temperature below the said predetermined temperature. 120

3. The improvement in the art of preparing paving material which comprises comminuting crude Trinidad asphalt, washing in water to remove soluble salts, adding thereto a refractory powder adapted to pre- 130

- vent granular adhesion, and drying by the application of heat thereby providing an asphalt having a granular structure.
4. The improvement in the art of preparing paving material which comprises comminuting crude Trinidad asphalt, washing said asphalt, and drying at a sufficiently low temperature to maintain the asphalt in granular form, then mixing the same cold with hot crushed mineral matter.
5. The improvement in the art of preparing paving material which comprises comminuting crude Trinidad asphalt, washing said asphalt in water and drying at a sufficiently low temperature to maintain the asphalt in granular form, then adding thereto a petroleum flux, and mixing at ordinary temperatures with proper proportions of hot sand and other reduced mineral matter.
- 20 6. The improvement in the art of preparing paving material which comprises comminuting crude Trinidad asphalt, subjecting the same to a drying process embodying an application of heat at a sufficiently low temperature to maintain the asphalt in granular form; then mixing in granular form, at a relatively low temperature, with fine heated mineral matter and a petroleum flux.
- 30 7. The improvement in the art of preparing paving material which comprises comminuting crude Trinidad asphalt, drying the same by the application of heat at a sufficiently low temperature to maintain the asphalt in granular form, then mixing in granular form, at a relatively low temperature, with hot sand and a petroleum flux.
- 40 8. The improvement in the art of preparing paving material which comprises comminuting crude Trinidad asphalt, adding thereto an agent adapted under ordinary conditions of handling to prevent granular adhesion, and subjecting same to a drying process at a sufficiently low temperature to maintain the granular condition thereof, adding thereto a petroleum flux and mixing cold with hot fine mineral matter.
- 50 9. The improvement in the art of preparing paving material which comprises comminuting crude Trinidad asphalt, washing said asphalt in water, adding thereto an agent adapted to prevent granular adhesion, drying by the application of heat, adding thereto a petroleum flux, and mixing cold with proper quantities of hot sand and 55 crushed mineral matter.
10. The improvement in the art of preparing paving material which comprises comminuting crude Trinidad asphalt, washing said asphalt, adding thereto an agent adapted to prevent granular adhesion, drying, adding thereto a petroleum flux, and mixing cold with hot sand or other fine mineral matter.
- 15 11. The improvement in the art of preparing bituminous cement which comprises comminuting crude Trinidad asphalt, adding thereto an agent adapted under ordinary conditions of handling at all temperatures below a certain predetermined temperature, to prevent granular adhesion, and 70 drying by the application of heat at a temperature below the said predetermined temperature.
- 25 12. The improvement in the art of preparing bituminous concrete which comprises comminuting crude Trinidad asphalt, drying by applying heat at a sufficiently low temperature to preserve the granular condition thereof, adding a solvent thereto and 80 mixing at ordinary temperatures with mineral matter.
- 35 13. The improvement in the art of preparing paving material, which comprises comminuting crude Trinidad asphalt and subjecting said asphalt to a drying process, embodying an application of heat, employing the heating medium at a temperature adapted to preserve the granular condition 85 of the asphalt.
- 45 14. The improvement in the art of preparing paving material which comprises comminuting crude Trinidad asphalt, subjecting said asphalt to a drying process embodying an application of heat at a temperature 95 adapted to preserve the granular condition of the asphalt, and mixing the same with hot crushed mineral matter.
- In testimony whereof we affix our signatures, in the presence of two witnesses.
- JAMES A. W. PINE.  
WILLIAM B. RUGGLES.
- Witnesses:  
LAURA E. SMITH,  
ARCHIBALD K. TOWERS.

Corrections in Letters Patent No. 1,057,667.

It is hereby certified that in Letters Patent No. 1,057,667, granted April 1, 1913, upon the application of James A. W. Pine and William B. Ruggles, of New York, N. Y., for an improvement in "The Art of Treating Asphalt," errors appear in the printed specification requiring correction as follows: Page 2, line 47, strike out the syllables "tended" and insert the words *or the mineral matter with which it is intended*; same page, strike out line 49, as now numbered; and that the said Letters Patent should be read with these corrections therein that the same may conform to the record of the case in the Patent Office.

Signed and sealed this 20th day of May, A. D., 1913.

[SEAL.]

C. C. BILLINGS,  
*Acting Commissioner of Patents.*